

M. McMURRAY, B. J. MULLEN & H. PEPPEL.

METHOD OF TREATING ORE.

APPLICATION FILED OCT. 14, 1913.

1,183,891.

Patented May 23, 1916.



Witnesses:  
Herman Eisele  
Nathan F. Trotter

Inventors:  
Max McMurray, B. J. Mullen and H. Peppel,  
By A. E. Merkel,  
their Attorney

# UNITED STATES PATENT OFFICE.

MAX McMURRAY, OF CLEVELAND, AND BENJAMIN J. MULLEN AND HARRY PEPPEL, OF LEETONIA, OHIO; SAID MULLEN AND SAID PEPPEL ASSIGNS TO UNITED IRON AND STEEL COMPANY, OF CLEVELAND, OHIO, A CORPORATION OF PENNSYLVANIA.

## METHOD OF TREATING ORE.

1,183,891.

Specification of Letters Patent. Patented May 23, 1916.

Application filed October 14, 1913. Serial No. 795,069.

To all whom it may concern:

Be it known that we, MAX McMURRAY, BENJAMIN J. MULLEN, and HARRY PEPPEL, citizens of the United States, residents, respectively, of Cleveland, county of Cuyahoga, and State of Ohio, and Leetonia, county of Columbiana, and State of Ohio, have invented a new and useful Improvement in Methods of Treating Ore, of which the following is a specification, the principle of the invention being herein explained and the best mode in which we have contemplated applying that principle, so as to distinguish it from other inventions.

Our invention relates to methods of treating ore and particularly to methods of treating ores which are in a finely divided or pulverulent state, such as, for instance, flue dust from blast furnaces.

The object of our invention is to provide a simple, economical and efficient method of treating such pulverulent ore, whereby it may be given physical characteristics such as will render it amenable from a commercial standpoint, to ordinary and well-known treatment designed to recover its valuable content.

As is well-known to those skilled in the art, one of the methods by which blast furnace flue-dust is rendered capable of such treatment, is called the "sintering-process". In the practice of this process, the pulverulent flue-dust is placed upon a porous hearth suitably supported, ignited so as to start internal combustion, that is combustion of the coke dust and sulfur content, and such combustion maintained by passing a current of air downwardly through the ore mass. The temperature which results from such combustion is such as will effect a partial fusing of the ore with a resultant agglomeration or sintering of the particles, so as to produce lumps of such character as will permit them to retain their integrity to such an extent, as to render them suitable for forming part of the charge of blast furnace, and permit their values to be extracted by the action of the latter.

In the sintering process as at present practised, grate-bars are used to support the porous hearth and the temperature generated is such as to eventually burn out these bars. In addition, it is necessary to em-

ploy means for creating the required air-current, which means usually consist of an exhaust fan or siphon. The ore mass is sometimes first moistened with water, as for instance, in a concrete mixer, whereupon it is placed upon its porous bed and an air current caused to flow therethrough. The mass is then ignited by means of a gas flame or by means of burning crude-oil previously sprayed upon its upper surface. This initial ignition shortly starts the combustion of the coke-dust in the mass and the sulfur of the iron-ore. The combustion so initiated is allowed to continue until the conversion or sintering is completed, whereupon the agglomerated mass is removed and broken up as desired.

The moistening of the dust, as above described, is resorted to in order to cause the particles to adhere to each other and permit the material to be more advantageously handled as well as to prevent it from too freely passing into the porous bed. In the present practice, this moisture is converted into steam in the initial part of the sintering process, after which any effect the steam may have on the process is eliminated.

The final or resulting condition of the material depends very largely upon the rate at which the air flows through the mass. If it pass slowly, the resultant product is more or less granular and unfused. If passed through rapidly, it becomes partially fused or sintered as is required. It is therefore essential that the air be permitted to pass through the mass with a certain amount of freedom, or in other words a certain degree of permeability be maintained in the mass throughout the process.

It is also desirable, from the standpoint of economy, to carry out the process by reducing the volume of air required to a minimum in order to operate the exhausting apparatus on as low a vacuum as possible, thereby reducing the amount of power consumed to a minimum.

With these main objects in view, our invention consists of a method hereinafter fully described and particularly set forth in the claims.

The annexed drawing and the following description are used to set forth in detail a certain method embodying our invention,

the disclosed detailed method, however, constituting but one of various methods in which the principle of the invention may be employed.

5. In said annexed drawing:—Figure 1 is a plan of a well-known form of a sintering pan forming part of the complete apparatus by means of which our process may be practised. Fig. 2 is a longitudinal section 10 of such pan. Fig. 3 represents a side elevation, upon a reduced scale, of one of the grate bars.

In carrying out our improved process, as is now the general practice, a porous bed 15 or hearth 1 is first formed in the bottom of the pan, which bed is supported by suitable grate-bars 2 having openings 3 (shown in dotted lines) therethrough through which the air may pass. This porous bed is about 20 one-half inch in depth and usually consists of lime-stone screenings. Upon this bed is charged the pulverulent ore, previously moistened or not, as circumstances may dictate.

25 Below the grate-bars is an inclosed chamber 4 provided with outlets 5, 5, which are connected with any suitable exhausting apparatus such as an exhaust fan or siphon (not shown). The exhausting apparatus is now 30 put into operation so as to cause an air current to travel downwardly through all such interstices which exist in the mass and through which the air can find its way and combustion initiated as above described.

35 Sufficient heat is soon generated to ignite the coke-dust, if any, in the charge as well as the sulfur content of the ore itself. The continued combustion of these elements furnishes sufficient heat for effecting the agglomeration or sintering as required and as 40 has heretofore been obtained.

45 After the initial ignition has progressed sufficiently to permit sintering to begin, instead of permitting such sintering to proceed from this point on as has heretofore been the custom, we supply the mass throughout the remainder of the process, with water, or its equivalent, either continuously or intermittently, in suitable amount, such amount de-

50 pending upon the nature of the charge and being determined empirically. This water is applied to the surface of the ore by any suitable means, such as a hose or spray, and is at once converted into steam, which along 55 with the air and products of combustion, passes through the charge and exhausts along with such air and combustion products. We have found that this application of the water gives the following economical results.

60 First, it reduces the time required to convert the charge, from twenty-five to fifty percent, according to the nature of the material to be converted. Second, the resultant product is very much more uniform in 65 its character, than has heretofore been the

case. Third, the exhausting apparatus it is found, may be run at a lower vacuum than heretofore, and fourth, the burning out of the grate-bars is greatly retarded if not altogether eliminated.

70 The first result is obtained by reason of the fact that the steam is an element in establishing and maintaining a more marked permeability than has heretofore been obtained, so that combustion is freer and 75 completion of oxidation and sintering is hastened. This probably accounts for the second of the above-named results, namely, the greater uniformity in the character of the resultant product.

80 The application of the water also decreases the temperature at which the sintering is conducted below that which would exist as a result of the unmodified or normal combustion. This is accompanied by a cooling and 85 hence a contraction of the volume of air which passes through the mass. Such decrease in volume hence permits of the employment of a lower vacuum in the exhausting apparatus as above noted. The reduction of temperature so effected, we have 90 found reduces the temperature of the exhaust gases from 100 to 300 degrees Fahrenheit, so that the exhausting apparatus is operated under comparatively low temperature 95 conditions. Difficulties heretofore experienced in operating such apparatus, and chiefly in connection with the bearings, are hence eliminated.

99 The water being introduced directly upon the burning ore reduces at once the temperature of the ore by reason of the heat being abstracted directly from the bed of fuel. This tends to check at once throughout the ore any volatilization of reduced metal, or perhaps of the formed dioxide which might be carried, when volatilized, into the supporting bed and be deposited there, or might be carried farther in.

105 The decrease in temperature is responsible for the fourth of the above-named results, namely, the retarding or elimination of the burning out of the grate-bars.

110 In this manner, therefore, we are enabled to carry out the process of sintering pulverulent material in a manner more economical and more expeditious than has heretofore, insofar as we are aware been practised, and with results superior to those which are ordinarily obtained.

115 Having fully described our invention, what we claim and desire to secure by Letters Patent is:—

120 1. The method of sintering fine ore which consists in establishing said ore together with fuel in a layer or bed, igniting said ore, allowing ignition to proceed until sintering conditions have been established, and supplying then directly upon the ignited ore, water to modify the sintering.

2. The method of sintering fine ore which consists in establishing said ore together with fuel in a layer or bed, igniting said ore, allowing ignition to proceed until sintering conditions have been established, and supplying then directly upon the ignited ore, water in quantity sufficient to maintain sintering conditions.

3. The method of sintering fine ore which 10 consists in establishing said ore together with fuel in a layer or bed, igniting said ore, allowing ignition to proceed until sintering conditions have been established, and supplying then directly upon the ignited ore, a

liquid in quantity sufficient to maintain sintering conditions.

Signed by me, this 13th day of Sept., 1913.

MAX McMURRAY.

Attested by—

F. C. KETTRING,

R. C. FARQUHAR.

Signed by us, this 16<sup>th</sup> day of Sept., 1913.

BENJAMIN J. MULLEN.

HARRY PEPPEL.

Attested by—

E. V. WARREN,

FRIEDA CHELLIS.